

3,539,310

**HYDROCARBON GELLING PROCESS USING ALUMINUM SOAP THICKENERS WITH SURFACE ACTIVE AGENTS**

Leo Finkelstein, Aberdeen, and Sidney J. Magram and Leonard Cohen, Baltimore, Md., and William T. Gregory, Rushville, Ill., assignors to the United States of America as represented by the Secretary of the Army  
No Drawing. Filed June 8, 1955, Ser. No. 514,135  
Int. Cl. C10I 7/02

U.S. Cl. 44—7

9 Claims

The invention described herein may be manufactured and used by or for the Government of the United States of America for governmental purposes without the payment to us of any royalty thereon.

The invention relates to the thickening of gasoline by aluminum soaps.

Gasoline, thickened or gelled by small quantities (about 1 to 12%) of aluminum soaps of the higher carboxylic acids, is important as an incendiary in warfare. Various aluminum soaps have been used, the best known being "napalm," the aluminum soap of a mixture of oleic and naphthenic acids and coconut oil fatty acids disclosed and claimed in U.S. Pat. No. 2,606,107 to Louis F. Fieser. More recently, improved results have been obtained by the use of about 0.75 to 4% of aluminum octoates, notably aluminum hydroxy di-(2-ethyl hexoate) and the iso-octoates disclosed in applications, Ser. Nos. 321,747 and 466,242, filed Nov. 20, 1952 and Nov. 1, 1954, respectively, by Leonard Cohen. These applications have matured into Pats. 2,741,629 and 2,718,462, respectively.

One advantage of these thickened gasolines over other incendiary fuel lies in the fact that they may be produced in the field by mixing the dry soap with gasoline. The proper amount of soap is added to a batch of gasoline and the mixture agitated until thickening occurs. The gel is then allowed to stand, or "cure," for a certain length of time. During the curing period the gel develops elasticity.

It is desirable that the time of mixing, or "vortex time," and the "cure time" be as short as possible, particularly to make it possible to use continuous rather than batch mixing and prompt use of filled bombs or flamethrowers. It is also desirable that the gel be as high in consistency as possible for a given amount of thickening agent, that it be highly elastic, and that it be stable over a long period of time.

We have found that the vortex time and the cure time can be shortened while retaining or enhancing the other desirable qualities by adding to the gasoline, prior to the addition of the aluminum soap, a minor amount of non-ionic surface-active agent, and that particular improvement can be obtained by the further addition, together with the surface-active agent, of certain small amounts of water. The improvement is particularly marked when the soap is aluminum hydroxy di-(2-ethyl hexoate).

While we do not wish to be bound by theory, we believe the explanation of the improved results to be as follows. In the process of formation of aluminum soaps by aqueous metathesis from sodium soap and aluminum salts in the presence of excess sodium hydroxide, aluminum hydroxide is formed together with the aluminum soap. This aluminum hydroxide is hydrophilic in nature and obstructs access of the hydrocarbons to the aluminum soap, thereby retarding gelation. It is believed that the addition of surface-active agents containing water causes hydration and addition by chemisorption of the lipophilic agent to the surface of the aluminum hydroxide, thereby eliminating the obstruction of access to the aluminum soap by the hydrocarbon solvents.

Generically, these nonionic surface-active compounds comprise a relatively large hydrocarbon group coupled to

a hydrophilic group which is nonpolar. Suitable hydrophilic groups are hydroxy, polyhydroxy, and polyoxethylene. The hydrocarbon and hydrophilic groups should be so balanced that the compound is readily soluble in hydrocarbons in the proportions employed and, for ease in preparing the gel, it is desirable that the compounds be liquid. While the entire genus of non-ionic surface-active agents appears to be usable, we have found the subgenus consisting of those containing the polyoxethylene group to be definitely superior in that they combine to the highest degree the various desirable properties set out above.

As stated earlier, we have found that further improvement in the vortex time and cure time is produced by employing water together with the surface-active agent. While commercial forms of the surface-active agents frequently contain varying amounts of water, we have found that optimum results are secured by the use of a narrow critical range of ratios of water to agent, extending from 10:90 to 15:85, by weight.

In order to secure mutual solubility of water and agent over a wide temperature range, it has been found desirable to employ a cosolvent such as isopropanol or the diethyl ether of diethylene glycol. A blend of water, agent, and cosolvent is prepared and then added to the gasoline or other hydrocarbon.

Suitable blends may contain the following ingredients in parts by weight:

|            |     |     |
|------------|-----|-----|
| Agent:     | 85  | 90  |
| Water:     | 15  | 10  |
| Cosolvent: | 100 | 100 |

A ratio of ten parts aluminum soap to one part of such a wetting agent blend has proved effective in the preparation of hydrocarbon gels ranging from 0.75 to 4% by weight of aluminum soap.

When all the desired characteristics are taken into account, two of the most desirable surface-active agents employed to date are:

| Trade name:  | Chemical nature                                                                 |
|--------------|---------------------------------------------------------------------------------|
| Triton X-45  | Octylphenoxyethoxy ethanol (average of about 5 ethoxy groups).                  |
| Atlas G-1256 | Polyoxethylene sorbitol esters of mixed fatty and resin acids (tall oil acids). |

The following examples illustrate the improvement attained by use of our invention.

**EXAMPLE I—(Control)**

In a laboratory mixer, four percent of aluminum hydroxy di-(2-ethyl hexoate), which had been formed by reacting aluminum sulfate or aluminum chloride with sodium 2-ethyl-hexoate in an aqueous solution of sodium hydroxide, was added to gasoline and the electric stirrer rotated at a fixed speed. As the mixture thickens, the level of the vortex rises about the rod of the stirrer. The time was noted for the level to rise from a predetermined initial level to a fixed point on the rod. This time is used as the vortex time. While the test is empirical in its choice of conditions, it is useful because it gives a quantitative measure of the time a thickener must be mixed in the field before it is allowed to stand or cure. The cure time was then determined by allowing the mixture to stand and noting the point at which elasticity developed.

On a series of tests as described above, the following results were secured:

Vortex time—20 to 40 minutes  
Cure time—>24 hours  
Gardner consistency after 24 hrs.—205

**3**  
**EXAMPLE II**

The tests were repeated as described in Example I, except that there was first added to the gasoline one part of a surface-active agent/water/cosolvent blend as described above for each ten parts of aluminum soap, and the soap was then introduced.

In a series of tests, using Atlas G-1256 and Triton X-45 as the agent, the following results were obtained:

Vortex time—less than 3 minutes

Cure time—about 15 minutes

Gardner consistency after 24 hrs.—650 to 700

In addition, the resulting gels were of higher consistency than obtained after a 24-hour cure in Example I.

Tables A thru D of the following tables of data show the suitability of other agents of the preferred subgenus, i.e. those containing the polyethoxy group.

Similar improvement has been noted when the non-ionic surface-active agents are used together with other aluminum soaps, including napalm and the isoocatoates disclosed in the application referred to above.

**TABLES OF DATA**

[Gasoline plus: 4% aluminum hydroxy di(2-ethyl hexoate) in gasoline, 0.1% surface-active agent—non-ionic]

| Trade name                                                                                                                                                         | Chemical nature                                         | Vortex time,<br>minutes<br>(at 77 F.) |
|--------------------------------------------------------------------------------------------------------------------------------------------------------------------|---------------------------------------------------------|---------------------------------------|
| (A) Polyoxyethylene sorbitan and sorbitol fatty acid derivatives                                                                                                   |                                                         |                                       |
| Tween 85                                                                                                                                                           | Polyoxyethylene sorbitan trioleate                      | 4.0                                   |
| Tween 81                                                                                                                                                           | Polyoxyethylene sorbitan monooleate                     | 2.25                                  |
| Tween 80                                                                                                                                                           | do                                                      | 3.0                                   |
| Tween 65                                                                                                                                                           | Polyoxyethylene sorbitan tristearate                    | 4.5                                   |
| Tween 60                                                                                                                                                           | Polyoxyethylene sorbitan monostearate                   | 3.3                                   |
| Tween 40                                                                                                                                                           | Polyoxyethylene sorbitan monopalmitate                  | 2.8                                   |
| Tween 20                                                                                                                                                           | Polyoxyethylene sorbitan monolaurate                    | 3.5                                   |
| Atlas G-2854                                                                                                                                                       | Polyoxyethylene sorbitol tetraoleate                    | 5.5                                   |
| Atlas G-2855                                                                                                                                                       | Polyoxyethylene sorbitol pentaoleate                    | 7.5                                   |
| (The preferred agent Atlas G-1256 is closely related to this group)                                                                                                |                                                         |                                       |
| (B) Alkyl polyoxyethylene alcohols                                                                                                                                 |                                                         |                                       |
| Esso-142                                                                                                                                                           | C <sub>10</sub> oxo alcohol—4.5 moles ethylene oxide    | 4.5                                   |
| Esso-154                                                                                                                                                           | C <sub>10</sub> oxo alcohol—6.6 moles ethylene oxide    | 8.9                                   |
| Esso-155                                                                                                                                                           | C <sub>10</sub> oxo alcohol—9.3 moles ethylene oxide    | 9.9                                   |
| Esso-141                                                                                                                                                           | C <sub>12</sub> oxo alcohol—3.3 moles ethylene oxide    | 6.0                                   |
| Esso-140                                                                                                                                                           | C <sub>12</sub> oxo alcohol—5.2 moles ethylene oxide    | 5.5                                   |
| Esso-139                                                                                                                                                           | C <sub>12</sub> oxo alcohol—ca. 12 moles ethylene oxide | 5.2                                   |
| Esso-153                                                                                                                                                           | C <sub>8</sub> oxo alcohol—5.9 moles ethylene oxide     | 7.1                                   |
| (C) Alkyl-aryl polyether alcohols                                                                                                                                  |                                                         |                                       |
| Igepal CO-630                                                                                                                                                      | Alkyl phenoxy polyoxyethylene ethanol                   | 3.8                                   |
| Igepal CA-630                                                                                                                                                      | do                                                      | 4.0                                   |
| Igepal CO-730                                                                                                                                                      | do                                                      | 4.0                                   |
| Oxonite dispersant NI-C                                                                                                                                            | Alkyl phenyl polyethoxyethanol                          | 3.5                                   |
| Triton X-155                                                                                                                                                       | Alkyl aryl polyether alcohol                            | 3.8                                   |
| Triton X-100                                                                                                                                                       | do                                                      | 3.8                                   |
| Tergitol-NPX                                                                                                                                                       | Alkyl phenyl polyethylene glycol ether                  | 2.8                                   |
| Tergitol-TMN                                                                                                                                                       | Alkyl ether of polyethylene glycol                      | 3.0                                   |
| Tergitol-CW                                                                                                                                                        | Alkyl aryl polyglycol ethers                            | 2.7                                   |
| (The preferred agent Triton X-45 belongs to this group. It contains fewer ethoxy groups than the other members and is therefore more readily soluble in gasoline.) |                                                         |                                       |
| (D) Aliphatic polyoxyethylene ether type                                                                                                                           |                                                         |                                       |
| Sterox AJ                                                                                                                                                          | Aliphatic polyoxyethylene ether type                    | 3.0                                   |
| Sterox SE                                                                                                                                                          | Aliphatic polyoxyethylene thio ether                    | 3.7                                   |
| Sterox SK                                                                                                                                                          | do                                                      | 4.0                                   |
| The following non-ionic agents not belonging to the preferred subgenus were also found to be operative                                                             |                                                         |                                       |
| (E) Sorbitan fatty-acid derivatives                                                                                                                                |                                                         |                                       |
| Span 80                                                                                                                                                            | Sorbitan monooleate                                     | 5.0                                   |
| Span 60                                                                                                                                                            | Sorbitan monostearate                                   | 1.8                                   |
| Span 40                                                                                                                                                            | Sorbitan monopalmitate                                  | 2.3                                   |
| Span 20                                                                                                                                                            | Sorbitan monolaurate                                    | 2.7                                   |
| Arlacel                                                                                                                                                            | Sorbitan sesquioleate                                   | 3.0                                   |
| (These gave satisfactory results, but are solids, requiring a dissolving step before addition of the soap.)                                                        |                                                         |                                       |
| (F) Higher alcohols                                                                                                                                                |                                                         |                                       |
| Hexanol                                                                                                                                                            |                                                         | 4.9                                   |
| Undecanol                                                                                                                                                          |                                                         | 4.8                                   |
| Pentadecanol                                                                                                                                                       |                                                         | 4.0                                   |
| Heptadecanol                                                                                                                                                       |                                                         | 3.5                                   |

While we have disclosed our invention in considerable detail, it will be appreciated that various changes are possible. We therefore wish our invention to be limited solely by the scope of the appended claims.

We claim.

1. A process of gelling gasoline comprising adding to

**4**

said gasoline a nonionic surface active agent selected from the group consisting of polyoxyethylene sorbitol esters of mixed tall oil acids, octylphenoxy polyethoxy ethanol and higher fatty acid derivatives of polyoxyethylene sorbitan, then adding an aluminum hydroxy soap of at least one higher carboxylic acid selected from the group consisting of higher fatty acids and mixtures of higher fatty acids and naphthenic acids, the amount of said soap being about one to twelve percent by weight of the gasoline and the amount of surface active agent being about five percent by weight of said soap, stirring the mixture of gasoline, soap and agent until it thickens and finally allowing the thickened mixture to stand until it develops elasticity.

2. A process as defined in claim 1 wherein the surface-active agent consists essentially of a higher fatty acid derivative of polyoxyethylene sorbitan.

3. A process as defined in claim 1 wherein said

surface-active agent consists essentially of polyoxyethylene sorbitol esters of mixed tall oil acids.

4. A process as defined in claim 1 wherein said surface-active agent consists essentially of octylphenoxy polyethoxy ethanol having an average of about five ethoxy groups to the molecule.

5. A process as defined in claim 1 wherein water is added together with said agent, the ratio of water to agent ranging from 10:90 to 15:85.

6. A process as defined in claim 2 wherein water is added together with said agent, the ratio of water to agent ranging from 10:90 to 15:85.

7. A process as defined in claim 3 wherein water is added together with said agent, the ratio of water to agent ranging from 10:90 to 15:85.

8. A process as defined in claim 4 wherein water is added together with said agent, the ratio of water to agent ranging from 10:90 to 15:85.

9. A process as defined in claim 1 in which the aluminum soap is aluminum hydroxy di-(2-ethyl hexoate).

## References Cited

## UNITED STATES PATENTS

|             |         |        |       |         |
|-------------|---------|--------|-------|---------|
| 2,390,609   | 12/1945 | Minich | ----- | 252—316 |
| 2,492,173   | 12/1949 | Mysels | ----- | 44—7 X  |
| 5 2,606,107 | 8/1952  | Fieser | ----- | 44—7    |
| 2,718,462   | 9/1955  | Cohen  | ----- | 44—7    |

## FOREIGN PATENTS

|         |        |                |
|---------|--------|----------------|
| 544,729 | 4/1942 | Great Britain. |
|---------|--------|----------------|

BENJAMIN R. PADGETT, Primary Examiner

U.S. Cl. X.R.

149—109